



US007183361B2

(12) **United States Patent**  
**Toman**

(10) **Patent No.:** **US 7,183,361 B2**  
(45) **Date of Patent:** **Feb. 27, 2007**

(54) **RHEOLOGY MODIFYING AGENTS AND METHODS OF USING THE SAME**

(75) Inventor: **Alan Toman**, Apex, NC (US)

(73) Assignee: **Reichhold, Inc.**, RTP, NC (US)

(\*) Notice: Subject to any disclaimer, the term of this patent is extended or adjusted under 35 U.S.C. 154(b) by 98 days.

(21) Appl. No.: **10/952,636**

(22) Filed: **Sep. 29, 2004**

(65) **Prior Publication Data**

US 2005/0069799 A1 Mar. 31, 2005

**Related U.S. Application Data**

(60) Provisional application No. 60/506,981, filed on Sep. 29, 2003.

(51) **Int. Cl.**  
**C08F 20/62** (2006.01)

(52) **U.S. Cl.** ..... **525/437; 525/438**

(58) **Field of Classification Search** ..... **525/437, 525/438**

See application file for complete search history.

(56) **References Cited**

**U.S. PATENT DOCUMENTS**

5,089,547 A 2/1992 McCabe et al.

|               |         |                           |
|---------------|---------|---------------------------|
| 5,241,019 A   | 8/1993  | Otsuki et al.             |
| 5,418,301 A * | 5/1995  | Hult et al. ..... 525/437 |
| 5,462,829 A   | 10/1995 | Tyagi et al.              |
| 5,780,195 A   | 7/1998  | Navia                     |
| 6,114,489 A   | 9/2000  | Vicari et al.             |
| 6,238,836 B1  | 5/2001  | Nakamura et al.           |
| 6,258,896 B1  | 7/2001  | Abuelyaman et al.         |
| 6,444,758 B2  | 9/2002  | McNamara et al.           |

**FOREIGN PATENT DOCUMENTS**

JP 07-219272 8/1995

**OTHER PUBLICATIONS**

Notification of Transmittal of the International Search Report and The Written Opinion of the International Searching Authority, or the Declaration, corresponding to PCT/US2004/31849, mailed Mar. 23, 2006.

\* cited by examiner

*Primary Examiner*—Kriellion Sanders

(74) *Attorney, Agent, or Firm*—Myers Bigel Sibley & Sajovec, PA

(57) **ABSTRACT**

The present invention provides, rheology modifying agents that include crystalline polymers wherein crystallinity is provided by a linear long chain aliphatic carboxylic acid on a base polymer. Such crystalline polymers can either have a hyperbranched or dendritic structure or have a comb-like structure.

**8 Claims, 9 Drawing Sheets**



FIG. 1



FIG. 2



FIG. 3





FIG 4



FIG 5



FIG. 6



FIG. 7



FIG. 8



FIG. 9



Avrami equation:

$$X(t) = 1 - \exp(-kt^n)$$

10 % blend, 25 °C

$$n = 0.14$$

$$k = 0.55 \text{ sec}^{-n}$$

$$30 \text{ s} = 0.59$$

$$60 \text{ s} = 0.63$$

FIG. 10



Region A: Melt transition of crystalline hyperbranched polyester  
Region B: Glass transition of amorphous toner polyester

FIG. 11

## 1

RHEOLOGY MODIFYING AGENTS AND  
METHODS OF USING THE SAMECROSS-REFERENCE TO RELATED  
APPLICATIONS

This application claims the benefit of, and incorporates herein by reference in its entirety, the following United States Provisional Application: U.S. Provisional Application No. 60/506,981, filed Sep. 29, 2003.

## FIELD OF THE INVENTION

This invention relates to rheology modifying agents, and particularly rheology modifying agents for toner applications.

## BACKGROUND OF THE INVENTION

Electrophotographic processes involve the transfer of an ink or toner image to a recording medium where the image is fixed. In typical electrophotographic processes, an electrostatic latent image is developed with toner and transferred to a recording medium, such as paper. The transferred toner image is fixed to the recording medium using known processes, such as by heating or fusing. Fixation of a toner image by heating typically involves the passing of a sheet of paper or other substrate containing toner particles through one or more fusing rollers. The heat applied by the fusing roller to the toner particles on the paper fixes the toner to the paper. The fixing of toner to paper or other substrates is well known.

One of the problems associated with the fixing of toner is the undesirable transfer of toner to the fusing roller during the fixing process. This undesirable transfer is sometimes referred to as "off setting" and involves the transfer of toner from the substrate to the fusing roller. The transfer of toner to the fusing roller contaminates the fusing roller, which results in the unwanted transfer of toner from the fusing roller onto subsequent substrates passing by the fusing roller. This transfer tends to produce ghost images or unwanted toner marks on subsequent substrates.

The off setting of toner to the fusing roller may be caused by a number of different factors. In some instances, toner is transferred to a fusing roller due to the cold offset or fixing temperature of the toner. The cold offset temperature is the temperature at which the toner begins to be fused. Typically, toners having lower viscosities have lower cold offset temperatures. In other instances, toner is transferred to the fusing roller because the toner loses its cohesive strength, producing a melted mass of toner that sticks to the fusing roller. The temperature at which this phenomenon occurs is known as the hot offset point or temperature. The hot offset temperature is related to the melt elasticity of the toner. Toners having lower melt elasticities exhibit lower hot offset temperatures whereas toners with higher melt elasticities have higher hot offset temperatures.

The difference between the hot offset temperature and the cold offset temperature is sometimes called the offset latitude, or a temperature range within which a fusing roller must operate in order to prevent off setting. In many toner fixing applications, the larger the offset latitude of the toner the better because a larger offset latitude provides a greater operational temperature range for the fusing rollers. Furthermore, a reduction in the cold offset temperature allows a decrease in the operational temperature of the fusing roller, which decreases the temperature in an electrophotographic apparatus, prolonging its life.

## 2

It is therefore desirable to develop toner compositions having greater offset latitudes. This can be accomplished by developing toner compositions having lower cold offset temperatures and higher hot offset temperatures.

5

## SUMMARY OF THE INVENTION

The present invention relates to rheology modification resins or polymers that may be added to various resin 10 compositions used in electrophotographic and printing processes.

According to embodiments of the present invention, rheology modifying agents include crystalline polymers wherein crystallinity is provided by a linear long chain 15 aliphatic carboxylic acid on a base polymer. Such crystalline polymers can either have hyperbranched or dendritic structures or have comb-like structures.

In one embodiment, the base polymer comprises a 20 branching monomer having a total functionality of three or more and an initiator monomer having at least two hydroxyl groups. The linear long chain aliphatic carboxylic acid is reacted with the initiator monomer to provide a crystalline polymer having a hyperbranched or dendritic structure. In another embodiment, the base polymer is a backbone monomer having multiple (more than one) pendant epoxy groups, 25 e.g., an epoxy cresol novolac resin. The backbone monomer is reacted with the linear long chain aliphatic carboxylic acid to provide a crystalline polymer having a comb-like structure or comb-like branching.

Such hyperbranched or comb-like crystalline polymeric 30 rheology modifying agents are added to resin compositions (e.g., toner resins) used in electrophotographic and printing processes to alter the rheology of the particular resin compositions.

35

BRIEF DESCRIPTION OF THE DRAWING  
FIGURES

The invention can be more readily ascertained from the 40 following description of the invention when read in conjunction with the accompanying drawings in which:

FIG. 1 illustrates an exemplary reaction for producing a 45 hyperbranched polyester;

FIG. 2 illustrates an exemplary reaction of a hyperbranched polyester with a linear carbon chain to produce a 50 rheology modifying agent according to embodiments of the present invention;

FIG. 3 illustrates an exemplary reaction of an epoxy 55 novolac resin with a linear carbon chain to produce a rheology modifying agent according to embodiments of the present invention;

FIG. 4 illustrates a plot of viscosity data for a toner and toner compositions according to embodiments of the present 60 invention;

FIG. 5 illustrates a plot of storage modulus data for a toner and toner compositions according to embodiments of the present invention;

FIG. 6 illustrates a plot of re-crystallization data of 65 rheology modifying agents and toner compositions according to embodiments of the present invention;

FIG. 7 illustrates a plot of viscosity data for a toner and toner compositions according to embodiments of the present invention;

FIG. 8 illustrates a plot of storage modulus data for a toner and toner compositions according to embodiments of the present 70 invention;

FIG. 9 illustrates a plot of re-crystallization data of rheology modifying agents and toner compositions according to embodiments of the present invention;

FIG. 10 illustrates a plot of re-crystallization data of rheology modifying agents and toner compositions according to embodiments of the present invention;

FIG. 11 illustrates a plot of melt transition data and re-crystallization data of hyperbranched rheology modifying agents according to embodiments of the present invention;

#### DETAILED DESCRIPTION OF THE INVENTION

The present invention now will be described more fully hereinafter with reference to the accompanying drawings. This invention may be embodied in many different forms and should not be construed as limited to the embodiments set forth herein; rather, these embodiments are provided so that this disclosure will be thorough and complete, and will fully convey the scope of the invention to those skilled in the art.

The offset properties of toner compositions have been found to depend on the rheology properties of the toner composition. For instance, the fixing temperature, or cold offset temperature, of a toner composition is related to the complex viscosity of the toner composition. A decrease in the viscosity of a toner composition results in a decrease in the cold offset temperature of the toner composition. Similarly, the hot offset temperature is related to the melt elasticity or storage modulus of a toner composition. An increase in the melt elasticity corresponds to an increase in the hot offset temperature. The modification of the rheology properties of a toner composition can therefore alter the temperatures at which offsetting will occur with the toner composition.

Embodiments of the present invention involve agents for modifying the rheology of resin compositions used in electrophotographic or printing processes, e.g., resins for toner, ink jet print, phase change inks, offset lithography, gravure, screen printing, flexography and paper-like displays. The rheology modifying agents include polymers and/or resins that may be added to resin compositions to modify the rheology of the resin composition. For example, a rheology modifying agent according to embodiments of the present invention may be added to a toner composition to alter the viscosity and/or melt elasticity of the toner composition.

Rheology modifying agents according to some embodiments of the present invention may be blended with resins, such as toner resins, to form a resin composition. The addition of the rheology modifying agent may increase the offset latitude of the resin. According to some embodiments of the present invention, the rheology modifying agents increase the offset latitude of the resin composition by decreasing the cold offset temperature of the resin composition. The addition of a rheology modifying agent of the present invention to a toner resin can lower the viscosity of the resin composition required during fusing, thereby decreasing the cold offset temperature of the resin composition.

Rheology modifying agents according to other embodiments of the present invention may be used to alter the melt elasticity of a resin composition. For instance, a rheology modifying agent may be added to a toner resin composition to increase the melt elasticity of the resin composition, thereby increasing the hot offset temperature of the resin composition. In some instances, the addition of a melt elasticity modifying agent may also alter the viscosity of the

resin composition, while in other instances, the rheology modifying agent will not alter the viscosity or provide a minimal viscosity increase.

According to other embodiments of the present invention, a rheology modifying agent can be adapted to both increase the melt elasticity of a toner resin composition and decrease the viscosity of the toner resin composition. The addition of such a rheology modifying agent broadens the offset latitude of the resin composition to which it is added.

In general, the rheology modifying agents are crystalline polymers wherein crystallinity is provided by a linear long chain aliphatic carboxylic acid on a base polymer. Specifically, in one embodiment, the crystalline rheology modifying agent is provided by a branching monomer having a total functionality of at least three or more, an initiator monomer on the branching monomer and having at least two hydroxyl groups, and the linear long chain aliphatic carboxylic acid reactive with the initiator monomer. Exemplary branching monomers include dimethylolpropionic acid, dimethylolbutanoic acid, glycidol, 4,4-bis (oxiranylmethoxyphenyl) valeric acid and 4,4-bis (4'-hydroxyphenyl) pentanoic acid.

Exemplary initiator monomers having at least two hydroxyl groups include methoxy polyethylene glycol, polyethylene glycol, trimethylolpropane, ethoxylated trimethylolpropane, trifunctional polyethylene glycol, tris-hydroxyethyl isocyanurate, ethoxylated pentaerythritol, styrene-allyl alcohol polymers, and bisphenol/epichlorohydrin oligomers and mixtures thereof.

Hyperbranched polymers include polymers having branching structures that are produced by a sequence of step-growth or addition polymerization reactions. Dendritic polymers include polymers having identical branching structures. The formation or synthesis of hyperbranched and dendritic polymers may be accomplished by known methods, for example, by esterification, amidation, free radical polymerization, or ionic polymerization methods. Any number of branches may be created in the hyperbranched or dendritic polymers used with the invention, although between about 10 and about 20 branches are preferred for some embodiments of the present invention.

Moreover by selection of the carboxylic acid the rheology modifying agent can be a solid at room temperature.

Examples of linear long chain aliphatic carboxylic acid that may be used with embodiments of the present invention include those listed in Table 1.

TABLE 1

| Number of Carbons | Name          | Common Name | Melt Point (° C.) |
|-------------------|---------------|-------------|-------------------|
| 14                | Tetradecanoic | Myristic    | 54                |
| 15                | Pentadecanoic |             | 51                |
| 16                | Hexadecanoic  | Palmitic    | 63                |
| 17                | Heptadecanoic | Margaric    | 59                |
| 18                | Octadecanoic  | Stearic     | 70                |
| 19                | Nonadecanoic  |             | 68                |
| 20                | Eicosanoic    | Arachidic   | 75                |
| 21                | Heneicosanoic |             | 74                |
| 22                | Docosanoic    | Behenic     | 81                |
| 23                | Tricosanoic   |             | 79                |
| 24                | Tetracosanoic | Lignoceric  | 78                |
| 25                | Pentacosanoic |             |                   |
| 26                | Hexacosanoic  |             | 88                |
| 27                | Hepacosanoic  |             | 88                |
| 28                | Octacosanoic  |             | 93                |

For example, a core molecule of trimethylol propane is reacted with dimethylol propionic acid to form a hydroxylated hyperbranched polyester. An example of the reaction is

illustrated in FIG. 1. The hydroxylated hyperbranched polyester is reacted with stearic acid at about 230° C. as illustrated in FIG. 2. The reaction of the hydroxylated hyperbranched polyester with stearic acid produces a rheology modifying agent according to embodiments of the present invention.

Crystalline rheology modifying agents according to other embodiments of the present invention include crystalline comb-branched polymers. The crystalline comb-branched polymers used as rheology modifying resins include polymer backbones having comb-like branches or side chains. In some embodiments, the branches or side chains are formed from fatty acids, such as stearic acid, or other linear long chain aliphatic carboxylic acids.

The backbone polymers used to form the comb-branched rheology modifying agents of the present invention may be selected from any polymer compatible with toner compositions, and preferably have more than one pendant epoxy group. Exemplary polymer backbones having pendant epoxy groups include, but are not limited to, novolacs. For instance, epoxy novolac resins are known and used in toner compositions as described in U.S. Pat. No. 5,780,195, which is incorporated herein by reference in its entirety. In some embodiments, for example, the polymer backbones can be selected from epoxidized cresol novolacs, epoxidized phenol novolacs, styrene-allyl alcohol, addition polymers containing glycidyl methacrylate and/or allyl glycidyl ether monomer, and mixtures and blends thereof. Polyvinyl alcohol-stearic acids may also be used to form comb-branched rheology modifying agents according to embodiments of the present invention. An epoxy novolac resin may be reacted with a linear carbon chain having an even number of carbon atoms. For example, esterification reactions can be used to attach the long chains. Such reactions involve the reaction of the acid with an oxirane group and with a hydroxyl group. The reaction can be performed with or without a catalyst. Other polymer backbones having reactive repeating units could also be used, for example, polyvinyl alcohol or a (meth)acrylate polymer formed from predominately hydroxyl or glycidyl functional (meth)acrylate monomers. Other examples include glycidyl methacrylate, allyl glycidyl ether, 2-hydroxyethyl acrylate and methacrylate, hydroxyl propyl acrylate and methacrylate, allyl alcohol, ethoxylated and propoxylated allyl alcohol, and vinyl alcohol.

For example, the reaction of an epoxy novolac resin with stearic acid to form a rheology modifying agent according to embodiments of the present invention is illustrated in FIG. 3. An epoxidized cresol novolac resin, such as Epiclon N-680 manufactured by Dainippon Ink & Chemicals of Japan, can be reacted with stearic acid at a temperature of about 225° C. in the presence of a catalytic amount of butyl stannoic acid (BSA). The reaction forms a rheology modifying agent having an epoxy novolac resin backbone with comb-like branches formed from the stearic acid. Although the Epiclon N-680 is limited to n=4.5, other epoxy novolac resins can be used to form similar structures that may be used as rheology modifying agents according to the present invention. For instance, n may range from about 3 to about 9.

The crystalline rheology modifying agents according to embodiments of the present invention crystallize through the formation of intra-molecular assemblies and are not dependent upon the diffusion rate of the polymer chains. The intra-molecular crystallization mechanism is provided by the high concentration of crystalline moieties existing per linear chain of carbon atoms within the crystalline structures. The presence of the crystalline moieties helps to

5 maintain the physical stability of the crystalline rheology modifying agents. Furthermore, the crystalline rheology modifying agents exhibit low melt viscosities, which correspond to low glass transition temperatures ( $T_g$ ) and melting points. The lower melt viscosities help to improve fixing and decrease the cold offset temperature and properties of a resin composition to which the crystalline rheology modifying agents are added. The crystalline rheology modifying agents also exhibit high storage modulus because of their high 10 molecular weight. This helps to improve the hot offset performance of the crystalline rheology modifying agents and resin compositions to which they are added.

Other embodiments of the present invention include toner resin compositions. Toner resin compositions of the present 15 invention include toner compositions combined with or mixed with rheology modifying agents of the present invention. A typical toner composition comprises a toner resin, a colorant and an electrostatic carrier material. Exemplary toner resins are disclosed in U.S. Pat. Nos. 5,780,195, 20 5,061,588, 5,089,547 and 5,324,611, the disclosure of which are incorporated by reference in their entirety.

25 Additional additives known by the skilled artisan may be employed in the toner resin composition of the present invention including, for example, inhibitors, paraffins, lubricants, and shrink-reducing additives. Any of the various suitable percentages of these additives can be used in conjunction with the toner resin composition.

The toner resin composition typically includes a colorant. 30 Exemplary colorants include a red pigment (e.g., red iron oxide, cadmium red, red lead oxide, cadmium, mercury sulfide, permanent red 4R, lithol red, pyrazolone red, watchung red, calcium salt, lake red D, brilliant carmine 6B, eosine lake, rhodamine lake B, alizaline lake, brilliant carmine 3B, or the like); a green pigment (e.g., chrome green, 35 chrome oxide green, pigment green B, malachite green lake, fanal yellow green G, or the like); a blue pigment (e.g., Prussian blue, cobalt blue, alkali blue lake, victoria blue lake, phthalocyanine blue, metal-free phthalocyanine blue, phthalocyanine blue particle chlorine compound, fast sky blue, indanthrene blue BC, or the like); a magenta pigment (e.g., manganese violet, fast violet B, methyl violet lake, or the like); a yellow pigment (e.g., chrome yellow, zinc yellow, cadmium yellow, yellow oxide, mineral fast yellow, nickel titanium yellow, nables yellow, naphthol yellow S, 40 hansa yellow G, hansa yellow 10G, benzidine yellow G, benzidine yellow GR, quinoline yellow lake, permanent yellow, NCG, tartrazine lake, or the like); an orange pigment (e.g., chrome orange, molybdenum orange, permanent orange GTR, indanthrene brilliant orange RK, vulcan orange, pyrazolone orange benzidine orange G, indanthrene brilliant orange GK, or the like); or a black pigment (e.g., carbon black, acetylene black, lamp black, aniline black, or the like). Suitable colorants are also disclosed in U.S. Pat. No. 3,989,648 to Lenhard et al. and U.S. Pat. No. 5,162,187 45 to Lyons et al., the disclosure of which are incorporated herein by reference in their entirety. Mixtures of any of the colorants may be used. The toner resin composition preferably includes from about 1 to 20 percent by weight of colorant.

50 The toner resin composition can also include a charge control agent such as Nigrosine Base EX (available from Orient Kagaku K.K.); quaternary ammonium salt (P-51: available from Orient Kagaku K.K.); Nigrosine Bontron N-01 (available from Orient Kagaku K.K.); Sudatiefschwarz BB (Solvent Black 3, C.I. 26150), Fettschwarz HEN (C.I. No. 26150); Briliantspiritschwarz TN (available from Farben Fabriken Bayer A. G.); Zapanschwarz X (available from

Farberke Hechist A. G.); and an alkoxylated amine, alkyl amide, molybdc chelating agent and the like. Mixtures of any of the charge control agents may be used. Preferably, the toner resin composition includes about 1 to 5 weight percent of charge control agent.

The rheology modifying agents of the present invention can improve the performance of toner compositions by increasing the offset latitude of the composition and by improving the rheology properties of the toner composition, which improves the toner quality in high speed fixing systems. In addition, some embodiments of the rheology modifying agents of the present invention do not plasticize, thereby improving toner performance.

Various embodiments of the present invention are illustrated by the following Examples, which are provided for illustrative purposes and are not meant to limit the embodiments of the present invention in any way:

#### EXAMPLE 1

A hyperbranched rheology modifying agent according to the present invention was formed from trimethylol propane, dimethylolpropionic acid, and stearic acid. A hydroxylated hyperbranched polymer was formed by the esterification reaction of trimethylol propane with dimethylolpropionic acid in the presence of methanesulfonic acid (MSA) at a temperature of about 140° C. The hydroxylated hyperbranched polymer was reacted with stearic acid at a temperature of about 230° C. to form the hyperbranched rheology modifier according to the reaction scheme illustrated in FIG. 2. The hyperbranched rheology modifying agent included about 0.19 weight percent trimethylol propane, about 35.26 weight percent dimethylolpropionic acid, and about 64.55 weight percent stearic acid. For illustrative purposes, the hyperbranched rheology modifying agent is also referred to as RMA1.

Various rheology properties for the RMA1 sample were determined. The onset of melting for the RMA1 sample occurred at 46.4° C., while the peak melting point occurred at 49.8° C. The melting points were measured using a Perkin-Elmer DSC7. The viscosity of the RMA1 sample was measured at 14.4 Poise. The viscosity of the RMA1 sample was measured using a Brookfield CAP 2000 rheometer operating at 60° C. and 500 rpm.

Toner compositions employing the hyperbranched rheology modifying resin RMA1 were made and tested. Samples of a toner composition (FE-208 produced by Dainippon Ink & Chemicals of Japan) were mixed with various percentages of the RMA1 sample to create toner compositions having 5 percent, 10 percent and 20 percent by weight RMA1. The melt viscosities of the toner composition samples were determined using an ARES dynamic mechanical analyzer manufactured by TA Instruments. The results were plotted and are illustrated in FIG. 4. The viscosities of the toner compositions having 10 percent and 20 percent by weight of RMA1 are lower than the viscosity of the FE-208 toner composition alone.

The toner compositions employing 5 percent, 10 percent, and 20 percent by weight hyperbranched rheology modifying resin RMA1 in combination with toner FE-208 were also tested to determine the storage modulus value at different temperatures. The results of the tests are plotted in FIG. 5 and compared to the storage modulus values of the FE-208 toner alone. In each instance, the storage modulus values of the toner compositions with RMA1 rheology modifying agents were higher than the corresponding storage modulus value for the FE-208 alone. Therefore, the addition of

RMA1 rheology modifying agents to a toner composition, such as toner FE-208, increases the storage modulus of the mixture.

The recrystallization behavior of the RMA1 rheology modifying agent alone and in combination with the FE-208 toner at 25° C. was determined and is plotted in FIG. 6. The y-axis in FIG. 6 represents the percentage of crystallization of the compound, which is plotted against time on the x-axis. At a time of 100 seconds, it can be seen that the re-crystallization of a toner composition comprising FE-208 toner and 10 percent by weight of an RMA1 rheology modifying agent is about 84 percent. This represents rapid re-crystallization of the toner composition and indicates that the rheology modifying agent has regained essentially all of its crystallinity within the timeframe of the test.

The toner compositions comprising a mixture of FE-208 toner and RMA1 rheology modifying agents exhibited lower melt viscosities and higher storage modulus values than that of the FE-208 toner alone. The decreased viscosities correspond to lower cold offset temperatures and the increases storage modulus values correspond to higher hot offset temperatures. As a result, the toner compositions including RMA1 rheology modifying agents exhibit a larger offset latitude range. In addition, the toner compositions comprising the FE-208 toner and RMA1 exhibited the same glass transition temperatures ( $T_g$ ) as that of the toner FE-208 alone. Thus, the glass transition temperature of the amorphous polyester FE-208 toner is unaffected by the presence of the crystalline rheology modifying agent RMA1.

#### EXAMPLE 2

A crystalline comb-like rheology modifying agent according to the present invention was formed from Epiclon N-680 and stearic acid. Epiclon N-680 is an epoxidized creosol-novolac resin produced and sold by Dainippon Ink & Chemicals of Japan. The Epiclon N-680 was reacted with stearic acid in the presence of BSA at a temperature of about 225° C. according to the reaction scheme illustrated in FIG. 3. Initially the epoxy group reacts with stearic acid and generates a hydroxyl group. This hydroxyl group is then esterified with additional stearic acid, resulting in the rheology modifying agent. The crystalline comb-like rheology modifying agent included about 30.62 weight percent Epiclon N-680 and about 69.38 weight percent stearic acid. For illustrative purposes, the crystalline comb-like rheology modifying agent is also referred to as RMA2.

Various rheology properties for the RMA2 sample were determined. The onset of melting for the RMA2 sample occurred at 45.1° C., while the peak melting point occurred at 48.2° C. The melting points were measured using a Perkin-Elmer DSC7. The viscosity of the RMA2 sample was measured at 49.8 Poise. The viscosity of the RMA2 sample was measured using a Brookfield CAP 2000 rheometer operating at 60° C. and 500 rpm.

Toner compositions employing the crystalline comb-like rheology modifying resin RMA2 were made and tested. Samples of a toner composition (FE-208 produced by Dainippon Ink & Chemicals of Japan) were mixed with various percentages of the RMA2 sample to create toner compositions having 5 percent, 10 percent and 20 percent by weight RMA2. The melt viscosities of the toner composition samples were determined and plotted. The results of the melt viscosity tests are illustrated in FIG. 7. The viscosities of the toner compositions having 5 percent, 10 percent, and 20 percent by weight of RMA2 are lower than the viscosity of the FE-208 toner composition alone. Thus, when added to

FE-208, the RMA2 rheology modifying agent lowered the viscosity of the toner composition.

The toner compositions employing 5 percent, 10 percent, and 20 percent by weight hyperbranched rheology modifying resin RMA2 in combination with toner FE-208 were also tested to determine the storage modulus value at different temperatures. The results of the tests are plotted in FIG. 8 and compared to the storage modulus values of the FE-208 toner alone. In each instance, the storage modulus values of the toner compositions with RMA2 rheology modifying agents were higher than the corresponding storage modulus value for the FE-208 alone. Therefore, the addition of RMA2 rheology modifying agents to a toner composition, such as toner FE-208, increases the storage modulus of the mixture.

The recrystallization behavior of the RMA2 rheology modifying agent alone and in combination with the FE-208 toner was determined and is plotted in FIG. 9. The y-axis in FIG. 9 represents the percentage of crystallization of the compound, which is plotted against time on the x-axis. At a time of about 100 seconds, it can be seen that the re-crystallization of a toner composition comprising FE-208 toner and 10 percent by weight of an RMA2 rheology modifying agent is about 67 percent. This represents rapid re-crystallization of the toner composition.

The re-crystallization of the toner composition comprising FE-208 toner and 10 percent by weight RMA2 rheology modifying agent was also analyzed using the Avrami equation. The results are plotted in FIG. 10. As illustrated, most of the re-crystallization is complete within a normal processing time for toners. Thus, the RMA2 rheology modifying agent will not plasticize the amorphous polyester FE-208 toner, and will avoid processing problems and poor storage stability of the toner caused by plasticization.

The toner compositions comprising a mixture of FE-208 toner and RMA2 rheology modifying agents exhibited lower melt viscosities and higher storage modulus values than that of the FE-208 toner alone. The decreased viscosities correspond to lower cold offset temperatures and the increases storage modulus values correspond to higher hot offset temperatures. As a result, the toner compositions including RMA2 rheology modifying agents exhibit a larger offset latitude range. In addition, the toner compositions comprising the FE-208 toner and RMA2 exhibited the same glass transition temperatures ( $T_g$ ) as that of the toner FE-208 alone, which indicates that the glass transition temperature of the amorphous polyester FE-208 toner is unaffected by the presence of the crystalline RMA2 rheology modifying agent.

A comparison of the properties of the FE-208 toner with the FE-208 toner and rheology modifying agent blends of Examples 1 and 2 is shown in TABLE 2. In particular, the viscosity at 105° C. (n) and the storage modulus values ( $G'$ ) at 105° C. and 180° C. are shown for each toner composition. The toner compositions comprising FE-208 toner and a rheology modifying agent are designated by the amount of rheology modifying agent added to the FE-208 toner on a weight percentage basis.

TABLE 2

|          | n<br>(kP, 105° C.) | $G'$<br>(Pa, 105° C.) | $G'$<br>(Pa, 180° C.) |
|----------|--------------------|-----------------------|-----------------------|
| FE-208   | 79.0               | 429.6                 | 3.1                   |
| 5% RMA1  | 49.1               | 359.0                 | 7.6                   |
| 10% RMA1 | 51.3               | 436.1                 | 10.2                  |

TABLE 2-continued

|          | n<br>(kP, 105° C.) | $G'$<br>(Pa, 105° C.) | $G'$<br>(Pa, 180° C.) |
|----------|--------------------|-----------------------|-----------------------|
| 20% RMA1 | 36.3               | 279.6                 | 7.6                   |
| 5% RMA2  | 59.8               | 388.9                 | 4.9                   |
| 10% RMA2 | 53.8               | 562.8                 | 6.1                   |
| 20% RMA2 | 21.3               | 142.1                 | 9.1                   |

FIG. 11 illustrates a DSC characterization of the resin blends produced by Examples 1 and 2. The graph shows that the re-crystallization of the rheology modifying agent is essentially unaffected by the presence of the amorphous polyester toner (FE-208). In addition, the glass transition temperature of FE-208 toner is not decreased by the presence of the rheology modifying agent.

## EXAMPLE 3

A series of carboxylic acids that can be used in the production of rheology modifying agents according to embodiments of the present invention were tested to determine relationships between the melt point of the carboxylic acids and polymers made from the carboxylic acids. The melt points were measured using a DSC instrument. The results of the melting point tests are illustrated in Table 3.

TABLE 3

| Carboxylic Acid                   | Melt Point<br>of acid (° C.) | Melt Point<br>of HBPE (° C.) |
|-----------------------------------|------------------------------|------------------------------|
| Myristic ( $C_{14}$ )             | 58.1                         | 18.1                         |
| Palmitic ( $C_{16}$ )             | 66.4                         | 35.2                         |
| Stearic ( $C_{18}$ )              | 72.5                         | 48.8                         |
| Behenic ( $C_{22}$ )              | 80.4                         | 63.5                         |
| Hystrene 9022 ( $C_{20}/C_{22}$ ) | 71.4                         | 60.3                         |

The melt points of the pure carboxylic acids illustrate a linear relationship between the melt point of the carboxylic acid and the melt point of a polymer made using the carboxylic acid. The mixed acids (Hystrene 9022 available from Crompton Corporation, Philadelphia, Pa.) did not produce a linear relationship. The relationships determined indicate that carboxylic acids having melt points of about 58° C. or greater would be suitable for producing rheology modifying agents according to embodiments of the present invention.

## EXAMPLE 4

A series of hyperbranched polymers were produced and tested to determine  $T_g$  differences in the polymers. The results are shown in Tables 4 and 5.

TABLE 4

| Functionality<br>of core | Molecular weight<br>of core | HBPE<br>generation | $\Delta T_g$ (° C.)<br>(10%) |
|--------------------------|-----------------------------|--------------------|------------------------------|
| 60                       | 1                           | 350                | -13.4                        |
|                          | 1                           | 350                | -3.6                         |
|                          | 1                           | 350                | -1.8                         |
|                          | 1                           | 350                | -0.9                         |
|                          | 1                           | 750                | -3.1                         |
| 65                       | 1                           | 2000               | -5.8                         |
|                          | 1                           | 2000               | -3.4                         |
|                          | 1                           | 5000               | -6.4                         |

TABLE 4-continued

| Functionality of core | Molecular weight of core | HBPE generation | $\Delta T_g$ (° C.) (10%) |
|-----------------------|--------------------------|-----------------|---------------------------|
| 2                     | 400                      | 2               | -6.7                      |
| 2                     | 400                      | 6               | -1.2                      |
| 2                     | 3350                     | 4               | -8.0                      |
| 2                     | 3350                     | 6               | -2.3                      |
| 3                     | 134                      | 3               | -1.2                      |
| 3                     | 134                      | 4               | -1.2                      |
| 3                     | 134                      | 5               | -1.0                      |
| 3                     | 134                      | 6               | -1.2                      |
| 3                     | 270                      | 5               | -1.0                      |
| 3                     | 990                      | 5               | -1.3                      |
| 3                     | 3900                     | 5               | -1.7                      |
| 3                     | 3900                     | 6               | -1.2                      |

TABLE 5

| Functionality of core | Molecular weight of core | HBPE generation | $\Delta T_g$ (° C.) (10%) |
|-----------------------|--------------------------|-----------------|---------------------------|
| 1                     | 350                      | 3               | -6.1                      |
| 1                     | 350                      | 4               | -2.6                      |
| 1                     | 350                      | 5               | -1.6                      |
| 1                     | 350                      | 6               | -1.0                      |
| 1                     | 750                      | 3               | -10.5                     |
| 1                     | 750                      | 4               | -5.8                      |
| 1                     | 750                      | 5               | -3.1                      |
| 1                     | 750                      | 6               | -1.1                      |
| 2                     | 300                      | 3               | -1.6                      |
| 2                     | 300                      | 4               | -0.2                      |
| 2                     | 300                      | 5               | -0.5                      |
| 2                     | 300                      | 6               | -0.8                      |
| 2                     | 1000                     | 3               | -4.8                      |
| 2                     | 1000                     | 4               | -3.2                      |
| 2                     | 1000                     | 5               | -1.4                      |
| 2                     | 1000                     | 6               | -1.1                      |
| 3                     | 270                      | 3               | -0.3                      |
| 3                     | 270                      | 4               | -0.3                      |
| 3                     | 270                      | 5               | -1.1                      |
| 3                     | 270                      | 6               | 0.0                       |
| 3                     | 990                      | 3               | -2.1                      |
| 3                     | 990                      | 4               | -1.2                      |
| 3                     | 990                      | 5               | -1.1                      |
| 3                     | 990                      | 6               | -1.0                      |

The data in Tables 4 and 5 indicate that once the core or the generation of the hyperbranched polymer is 3 or greater, the molecular weight does not significantly affect the usability of the polymer.

In the drawings and specification, there have been disclosed embodiments of the invention and, although specific terms are employed, they are used in a generic and descriptive sense only and not for purposes of limitation. The following claims are provided to ensure that the present application meets all statutory requirements as a priority application in all jurisdictions and shall not be construed as setting forth the full scope of the present invention.

That which is claimed:

1. A composition for use in electrophotographic or printing processes, the composition comprising a resin composition suitable for such processes and a rheology modifying agent, said rheology modifying agent being a solid at room temperature and comprising a branching monomer having a total functionality of three or more, an initiator monomer having at least two hydroxyl groups, and a linear long chain aliphatic carboxylic acid reactive with said initiator monomer, said linear long chain aliphatic carboxylic acid is

selected from a group consisting of tetradecanoic acid, pentadecanoic acid, hexadecanoic acid, heptadecanoic acid, octadecanoic acid, nonadecanoic acid, eicosanoic acid, heneicosanoic acid, docosanoic acid, tricosanoic acid, tetracosanoic acid, pentacosanoic acid, hexacosanoic acid, hepacosanoic acid, and octacosanoic acid.

2. The composition of claim 1, wherein the branching monomer is selected from the group consisting of dimethylolpropionic acid, dimethylolbutanoic acid and glycidol.

10 3. The composition according to claim 1, wherein the initiator monomer having two or more hydroxyl groups is selected from the group consisting of methoxy polyethylene glycol, polyethylene glycol, trimethylolpropane, ethoxylated trimethylolpropane, trifunctional polyethylene glycol, tris-hydroxyethyl isocyanurate, ethoxylated pentaerythritol, styrene-allyl alcohol polymers, and bisphenol/epichlorohydric oligomers and mixtures thereof.

4. A composition for use in electrophotographic or printing processes, the composition comprising a resin compo-

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815